

# UNITED STATES PATENT OFFICE.

WALTER E. HASSAM, OF WORCESTER, MASSACHUSETTS, ASSIGNOR TO HASSAM PAVING COMPANY, A CORPORATION OF MASSACHUSETTS.

## METHOD OF MAKING ROADS, PAVEMENTS, AND THE LIKE.

1,215,273.

Specification of Letters Patent.

Patented Feb. 6, 1917.

No Drawing.

Application filed November 29, 1915. Serial No. 63,954.

*To all whom it may concern:*

Be it known that I, WALTER E. HASSAM, a citizen of the United States, residing at Worcester, in the county of Worcester and 5 State of Massachusetts, have invented a new and useful Method of Making Roads, Pavements, and the like, of which the following is a specification.

The principal object of this invention is 10 to provide an improved wearing surface for the type of pavement known as the Hassam pavement, of which I am the inventor.

Several types of surface coatings have been suggested and used, but for various 15 reasons they usually have to be placed on the Hassam pavement only after the cement grouting has dried and hardened, and the same condition prevails when these coatings were placed on pavements made of ordinary 20 cement concrete. Moreover it has proved practically impossible to make the old coatings absolutely impervious. Therefore water frequently gets down under them in places and freezes and thaws. This causes the top 25 or cover layer to heave and eventually become loosened in spots which causes the road to break down. Intense summer heat also softens the ordinary coatings and causes them to creep.

30 It is well known that most types of these pavements set in a stronger condition and are subject to less danger from fissures and cracks, so that they are more durable, if after the pavement is laid a coating of loam, 35 sand or other protecting material is applied and left for a period of about ten days to prevent the green pavement being subjected to the action of the sun, as well as the wind and rain. In fact in many States now the 40 specifications are systematically prepared in such a way as to necessitate the use of this method.

One of the objects of this invention is to 45 provide an improvement in the Hassam pavement which will permit of the application of the surface coating directly on the wet and plastic grouting the day it is laid without waiting for it to harden, and which will in itself constitute a protecting coating 50 during the drying and hardening of the grouting, so that the expense and delay necessitated by the above mentioned temporary covering process will be avoided.

55 I accomplish this result by making a pavement in the usual manner employed in lay-

ing the Hassam pavement, but instead of the surface treatments heretofore suggested I apply to the surface an emulsified bituminous coating in a cold condition while the grouting is in a wet and plastic state. More 60 specifically the method of procedure which I prefer is as follows:—

In the first place after excavating as usual, I spread a layer of aggregate material, preferably in the form of uncoated stone, on the 65 foundation and roll it in its dry state until it is compacted as much as possible, so that the voids are reduced materially. Then I apply to it a thin grouting of cement, sand and water in a creamy condition. This is 70 poured over the surface and allowed to sink down in and fill the voids and I supply enough so that it comes substantially to the surface of the layer of stone. As so far described I proceed according to the method 75 laid down in my own prior patents for the making of the so-called Hassam pavement, but while the grouting is in its wet state and while it is substantially at a uniform level I place upon it a layer formed of aggregate 80 material, emulsified bitumen and Portland cement, the aggregate material preferably involving broken stone and sand. The proportions may conveniently be as follows:—

Stone 12 parts, cement 1 part, sand six parts, 85 and sufficient bitumen about two parts to coat all the stone. These materials are thoroughly incorporated together so that the sand and stone are covered throughout their 90 surfaces by the mixture of emulsified bitumen and cement, and then a layer of this material in a cold state is placed on the wet surface of the grout, said layer being one or two inches thick or more as may be desired. Finally I roll the whole surface to 95 force the upper layer of broken stone into the grouting while the latter is still wet and before it has commenced to set. This is important, because if the grouting is disturbed after it has commenced to set it will set in 100 a weak condition and never have the strength and durability that it has when operated upon as above described. Furthermore, this last rolling forces the surface moisture out of the wet grouting directly up through the 105 bituminous layer. In this way the grouting starts to solidify at the time that the stones are forced into it and its moisture removed, so that thereafter it is free to solidify and harden without the expression of any ma- 110

terial further amount of moisture. Of course this rolling operation also solidifies the bituminous layer and furnishes a smooth hard surface for the road bed.

5 I am aware of the fact that it has been proposed before to use emulsified bitumen in combination with broken stone, sand and cement as a surface layer for an ordinary cement concrete pavement, but owing to the 10 fact that it has to be rolled in order to make it of value and the further fact that the cement concrete when in its plastic state cannot be rolled adequately so as to bring it to a uniform surface, that method has not 15 proved a practical one so far as I am aware. It is practical when applied in the way described herein because the first compacted stone layer is strong enough to stand the 20 passage of the heaviest road roller over it without forcing the stones out in front and at both sides as is the case with the cement concrete pavement.

By rolling the stone coated with emulsified asphalt and cement into the top of the 25 grouting while still in a receptive state as described above the setting of the grouting is materially modified. Instead of simply having its moisture evaporated into the air slowly and setting in a period of several 30 days by evaporation and gravity alone it is positively compacted. The grouting does not commence to set until after the excessive moisture is removed. In the ordinary manner this takes considerable time, but in this 35 case it is squeezed out by the rolling process and consequently its setting action is hastened. Furthermore as stated above, the bituminous coating layer applied at the time of placing the lower layer in position serves 40 as a protection during the hardening of the cement grouting, and consequently does away with the expensive and delaying operation of covering the pavement with a temporary protecting cover.

45 Among the other advantages of this invention are the following:—A top layer or wearing surface is provided which can be applied to a Hassam foundation so that said top layer will actually combine therewith—said top layer will be durable in all kinds of weather—said top layer will remain in its original position on the Hassam foundation after long usage—said top layer can be laid and repaired easily without skilled 50 labor—said top layer will not disintegrate to form dust—said top layer will have a good appearance—said top layer will make the pavement practically noiseless—said top layer can be laid on the Hassam foundation 55 in damp or even rainy or slightly freezing weather so that time can be saved under certain weather conditions—and said top layer will have substantially the same rate of expansion and contraction as the Hassam 60 foundation, whereby deterioration of the 65

pavement by reason of internal strains and stresses will be much reduced.

Another way in which the method can be carried out from the point at which the grouting is applied is as follows:—Over the 70 grouting can be applied a layer of uncoated broken stones and these can be rolled into the grouting. Then a mixture of emulsified bitumen, Portland cement and sand in a comparatively thin state can be poured over 75 the same and again rolled.

Although I have illustrated and described only two ways of proceeding I am well aware of the fact that other modifications in the manner of carrying out the process can be made without departing from the scope of the invention as expressed in the claims. Therefore I do not wish to be limited to all the details of procedure herein described, but what I do claim is:

80 1. The method of making a pavement or the like, which consists in spreading a layer of uncoated aggregate material, rolling it until the voids are small, applying to it a thin cement grouting until the voids are 90 filled and the grouting seeks its level substantially at the surface of said layer of aggregate material, then while said grouting is in its wet state and before its surface has been disturbed placing upon it a layer 95 formed of a mixture of aggregate material, emulsified bitumen, and Portland cement thoroughly incorporated together, and finally rolling.

100 2. The method of making a pavement or the like, which consists in spreading a layer of uncoated broken stone, rolling it until the voids are small, applying to it a thin cement grouting in a creamy state until the voids are 105 filled and the grouting rises to the top of the layer of stone, then before the grouting commences to set placing upon it a layer formed of a mixture of broken stone, emulsified bitumen, Portland cement, and sand thoroughly incorporated together, finally rolling to 110 force the upper layer of broken stone into the grouting while still wet, force the surplus moisture directly out of the grouting and up through the bituminous layer and solidify said bituminous layer.

115 3. The method of making a pavement or the like which consists in spreading a layer of dry, uncoated, broken stone on a foundation, rolling it to compact it throughout and bring its top surface into a uniform condition, pouring upon it a thin cement grouting in a creamy state until the voids among the stones are filled and the grouting rises substantially to the top of the stone layer, then before the grouting commences to set and 120 while in a liquid state, placing upon it in a cold state a thin layer formed of a mixture of broken stone, emulsified bitumen, Portland cement, and sand thoroughly incorporated together, and rolling to force the upper layer 125 130

into the grouting while still wet and before it has commenced to set.

4. The method of making a pavement or the like which consists in spreading a base layer of dry, uncoated, broken stone on a foundation, rolling it to compact it throughout and bring its top surface into a uniform condition, pouring upon it a thin cement grouting in a creamy state until the voids among the stones are filled, then placing upon said layer in a cold state a layer formed of a mixture of broken stone, emulsified bitumen, Portland cement, and sand, thoroughly incorporated together, and rolling to force the upper layer into the base layer while still wet.

5. A pavement having a base layer of

hard, rolled, uncoated stone and a grouting of cement filling the voids therein, and a top layer formed of a mixture of broken stone, 20 emulsified bitumen, Portland cement, and sand thoroughly incorporated together and united with the base layer.

6. A pavement having a base layer of hard, rolled, uncoated stone and a grouting 25 of cement filling the voids therein, and a top layer formed of about twelve parts broken stone, one part Portland cement, six parts sand, and two parts emulsified bitumen incorporated together and united with 30 the base layer.

In testimony whereof I have hereunto set my hand.

WALTER E. HASSAM.